

Nov. 27, 1956

J. R. WEST ET AL

2,772,153

ROASTING PYRITES

Filed Aug. 4, 1955

2 Sheets-Sheet 1



*Fig. 2.*

INVENTORS  
JAMES R. WEST, and  
FREDERICK GORMLEY

BY  
Brown, Codd, Dow, Price & Penman  
their ATTORNEYS

Nov. 27, 1956

J. R. WEST ET AL

2,772,153

ROASTING PYRITES

Filed Aug. 4, 1955

2 Sheets-Sheet 2



Fig. 3.



Fig. 4.

INVENTORS.  
JAMES R. WEST, and  
FREDERICK GORMLEY.

BY  
Brown, Hutchison, Price, Prohlem  
their  
ATTORNEYS.

1

2,772,153

## ROASTING PYRITES

James R. West, Pittsburgh, Pa., and Frederick Gormley, Vera Cruz, Mexico, assignors to Texas Gulf Sulphur Company, New York, N. Y., a corporation of Texas

Application August 4, 1955, Serial No. 526,460

7 Claims. (Cl. 75—9)

This invention relates to the roasting of pyrites, and a major object is to provide a method of roasting it to produce elemental sulfur (S) and ferric oxide ( $Fe_2O_3$ ).

Another object is to provide such a method in which inert gas is used to free the labile sulfur as the first step, or stage, of roasting with production of a minimal amount of sulfur dioxide ( $SO_2$ ).

Yet another object is to provide a method of the foregoing types in which roasting of the sulfur contained in pyrites is effected chiefly by means of sulfur dioxide.

As special object is to provide a method in accordance with the foregoing objects in which pyrrhotite ( $FeS$ ) is reacted with sulfur dioxide to produce magnetite ( $Fe_3O_4$ ) and elemental sulfur, and in which the sole source of sulfur dioxide is produced by reacting ferric oxide with pyrrhotite to produce magnetite and sulfur dioxide.

Still another object is to effect roasting of pyrites in accordance with the foregoing objects to produce ferric oxide containing less residual sulfur than has been the case with prior roasting methods.

A still further object is to effect roasting of pyrites in accordance with the foregoing objects under fluidizing conditions.

The invention will be described with reference to the accompanying drawings in which:

Fig. 1 is a schematic representation of one mode of practicing the invention;

Fig. 2 is a flow sheet representing one embodiment of the invention as practiced with fluidization;

Fig. 3 is a flow sheet illustrating another embodiment of the invention using fluidization; and

Fig. 4 is still another flow sheet representing yet another fluidized embodiment.

We have discovered, and it is upon this that the invention is largely predicated, that the stated objects of the invention are attained by treating pyrites with an inert gas that is non-oxidizing to sulfur, and preferably comprising essentially at least one member of the group consisting of nitrogen ( $N_2$ ) and sulfur dioxide at a temperature at which the labile sulfur atom is driven from the pyrites with formation of pyrrhotite, treating the resultant pyrrhotite with at least one member of the group consisting of oxygen ( $O_2$ ) and sulfur dioxide at a temperature to convert it to magnetite, heating the magnetite with an oxygen-containing gas at a temperature to convert it to ferric oxide, and recovering the sulfur produced and the ferric oxide produced.

Having reference now to the drawings, Fig. 1 shows schematically a reactor 1 in the form of a vertical moving bed shaft furnace into the upper end of which, as indicated in the drawing, pyrites is introduced through suitable feeding mechanism, not shown. The pyrites may suitably be in the form of lumps ranging in size from one-half inch to two or three inches in equivalent diameter. Air preheated sufficiently to cause the various reactions to occur is fed into the bottom of reactor 1 together with a mixture of sulfur dioxide and nitrogen originating as described hereinafter. In the upper end of the reactor the following reaction occurs



(1)

2

The pyrrhotite thus formed reacts, in moving down the shaft, with sulfur dioxide to produce magnetite according to the following reaction



Pyrrhotite likewise reacts with any oxygen remaining in the upmoving gases in accordance with the following reaction



10 The magnetite formed by either or both of Reactions 2 and 3 then reacts with the oxygen of the air introduced into the bottom of the reactor, as shown, according to the following reaction



15 There is withdrawn from the top of the furnace a mixture of sulfur dioxide, nitrogen and sulfur vapor, which is, as shown, passed to a sulfur condenser 2 of any suitable type. The residual mixture of sulfur dioxide and nitrogen is withdrawn from the condenser and a sufficient amount for the purposes of the foregoing reactions is recycled to the reactor 1 through a conduit 3, the remaining portion being passed at 4 to a stack. In the practice of this embodiment of the invention the air supplied to the reactor is controlled in an amount such as to effect Reaction 3 and to avoid having any substantial excess of oxygen passing into the upper portions of the reactor, whereby oxidation of the sulfur of the pyrites and pyrrhotite is avoided. In this way the maximum amount of sulfur is recovered as such.

20 Various modifications of the embodiment of Fig. 1 of the invention are permissible. For instance, the ferric oxide from reactor 1 may be passed to a chloridizing reactor into which common salt, air and fuel are introduced for conversion of non-ferrous metals, such as nickel and copper, present in the ore into soluble chlorides. Similarly, the excess sulfur dioxide from condenser 2 that is not required for circulation in the system may be passed to a liquefaction plant to recover sulfur dioxide for desired use. In this latter embodiment it may be preferable to supply oxygen instead of air to the bottom of shaft furnace 1 whereby there is no necessity for separating nitrogen from the sulfur dioxide that is to be liquefied.

25 In the preferred embodiment of the invention the various stages of the process are carried out under fluidizing conditions, as illustrated in Figs. 2 to 4. Referring to Fig. 2, pyrites in a form adapted to be fluidized is passed to a preheater 5 where it is fluidized by a stream of hot gas composed of nitrogen and sulfur dioxide from a heater 6, the temperature of the gas being such as to drive the labile sulfur atom from the pyrites and form pyrrhotite in accordance with Reaction 1. The pyrrhotite passes into reactor 7 where it is fluidized with a gas composed chiefly of oxygen and nitrogen at a temperature such as to cause Reactions 2 and 3 to occur. The resulting magnetite then passes to a reactor 8 where it is fluidized with air at a temperature to effect Reaction 4, with the off-gas (largely  $O_2$  and  $N_2$ ) being passed to reactor 7.

30 Pyrites is fed likewise to a preheater 5a where it is fluidized with hot gas from heater 6 with production of pyrrhotite according to Reaction 1. The pyrrhotite thus produced passes to a reactor 7a where it is fluidized with the mixture of sulfur dioxide and nitrogen from reactor 7, and by sulfur dioxide from heater 6, with production of magnetite and elemental sulfur. The magnetite from reactors 7 and 7a is then passed to reactor 8, where it is fluidized by air and from which ferric oxide, per Reaction 4, is withdrawn.

35 The mixture of sulfur dioxide, sulfur vapor and nitrogen from reactors 5 and 5a is passed to a sulfur condenser 9 of any desired type from which the sulfur is recovered, with the residual gas being passed to a stack

## 3

or to a sulfur dioxide liquefaction plant. The mixture of sulfur dioxide, nitrogen and sulfur vapor from reactor 7a is likewise passed to sulfur condenser 9a for recovery of its content of sulfur, the residual sulfur dioxide and nitrogen then being passed to heater 6 for recirculation in the system in the manner described.

Although preheater 5, reactor 7 and reactor 8 are shown in the flow sheet as separate units, it will be understood that the three stages may be combined in a single fluidized reactor with the top, middle and bottom zones being represented, respectively, by preheater 5, reactor 7 and reactor 8. Likewise, the same thing applies to preheater 5a and reactor 7a.

If desired, all or a portion of the ferric oxide from reactor 8 may be passed to a chloridizing reactor 10 in the manner and for the purpose described in connection with Fig. 1.

Having reference now to Fig. 3, here again pyrites of appropriate size is fed to a preheater 11 where it is fluidized with an inert gas from generator 12 at a temperature sufficient to drive the labile sulfur atom from the ore and form pyrrhotite. The inert gas supplied from generator 12 may be flue gas composed largely of nitrogen and carbon dioxide, or it may be blast furnace gas, or other gas that is substantially free from oxygen and nonreactive with sulfur under the roasting conditions. A portion of the pyrrhotite from preheater 11 then is fluidized in a reactor 13 with sulfur dioxide under conditions in accordance with Reaction 2, thus forming magnetite and elemental sulfur. Another portion of the pyrrhotite formed in preheater 11 is passed to a reactor 13a where it is fluidized with sulfur dioxide at a temperature to cause Reaction 2 to proceed, likewise with production of magnetite and sulfur vapor. The magnetite from reactors 13 and 13a then passes to a reactor 14 where it is treated at a temperature such that with oxygen or a gas containing a high percentage, say 85 to 95 percent, of oxygen, preferably in an amount such that the off-gas, if any, is substantially oxygen-free and consists essentially of nitrogen.

An important feature of this embodiment of the invention is the recirculation, as shown, of a portion of the ferric oxide from reactor 14 to reactor 13 where the following reaction occurs



Reaction 5 constitutes in this embodiment the sole source of the sulfur dioxide used in this embodiment, which is important and desirable in that oxidation of sulfur in reactors 13 and 13a and preheater 11 is avoided.

Ferric oxide from reactor 14 is withdrawn and passed to use or storage, and the mixture of inert gas and sulfur vapor from preheater 11 is passed to a suitable sulfur condenser 15 from which sulfur is withdrawn, with the inert gas being wasted. Similarly, the mixture of sulfur dioxide and sulfur vapor from reactors 13 and 13a are passed to a condenser 15a for recovery of the sulfur content, the sulfur dioxide from the condenser being passed to a heater 16 for recirculation to reactors 13 and 13a, as described.

As in the case of Fig. 2, the separate stages of preheater 11 and reactors 13 and 14 may be combined in a single fluidized unit.

The embodiment of Fig. 4 is generally similar to that of Fig. 3 in that pyrites of appropriate size is fluidized in preheater 17 with an inert gas at a temperature such as to drive off the labile sulfur atom which with the inert gas is passed to a condenser 19 for recovery of the sulfur. One portion of the pyrites from the preheater 17 passes to a reactor 18, and the other portion passes to a reactor 18a in each of which the pyrrhotite from 17 is fluidized with sulfur dioxide at a temperature to effect Reaction 2. The magnetite from the two reactors is then fluidized with air in a reactor 19 at a temperature to convert the magnetite to ferric oxide in accordance with

## 4

Reaction 4. In this embodiment the air is preferably supplied to reactor 19 in such an amount that the product gas consists essentially of nitrogen which is passed as the inert gas to preheater 17. Preferably, a portion of the ferric oxide leaving reactor 19 is recycled to reactor 18, as shown, for the purpose described in connection with Fig. 3. The mixture of sulfur dioxide and sulfur vapor from reactors 18 and 18a is passed to an appropriate condenser 21 for recovery of the sulfur, with the separated sulfur dioxide passing to a heater 22 whence it is fed to reactors 18 and 18a. Here, also, preheater 17 and reactors 18 and 19 may be combined in a single fluidized unit.

Although in various embodiments two sulfur condensers have been shown and described, it will be understood that all of the sulfur vapor-carrying gases may be treated in a single condenser. Likewise, in all instances the ferric oxide may go to a chloridizer, per Figs. 1 and 2.

According to the provisions of the patent statutes, we have explained the principle of our invention and have illustrated and described what we now consider to represent its best embodiment. However, we desire to have it understood that, within the scope of the appended claims, the invention may be practiced otherwise than as specifically illustrated and described.

We claim:

1. That method of roasting pyrites to produce sulfur and ferric oxide comprising fluidizing one portion of pyrites with nitrogen-containing gas substantially free from oxygen at a temperature to drive off the labile sulfur atom and form pyrrhotite, separately fluidizing a second portion of pyrites in the same manner, recovering the sulfur from said treatments, fluidizing the pyrrhotite from said one portion with an oxygen-containing gas at a temperature to convert it to magnetite and produce sulfur dioxide, fluidizing the pyrrhotite from said second portion with sulfur dioxide, including that from said one portion, at a temperature to convert the pyrrhotite to magnetite with production of a mixture of sulfur dioxide and sulfur vapor, condensing sulfur from said mixture and passing part of the residual sulfur dioxide to treat said one portion and passing another part to treat the pyrrhotite from second portion, uniting the magnetite thus produced and fluidizing it with an oxygen-containing gas at a temperature to convert it to ferric oxide, and recovering ferric oxide.

2. That method of roasting pyrites to produce sulfur and ferric oxide comprising fluidizing one portion of pyrites with nitrogen-containing gas substantially free from oxygen at a temperature to drive off the labile sulfur atom and form pyrrhotite, separately fluidizing a second portion of pyrites in the same manner, recovering the sulfur from said treatments, fluidizing the pyrrhotite from said one portion with an oxygen-containing gas at a temperature to convert it to magnetite and produce sulfur dioxide, treating the pyrrhotite from said second portion with sulfur dioxide, including that from said one portion, at a temperature and with fluidization to convert it to magnetite with production of a mixture of sulfur dioxide and sulfur vapor, condensing sulfur from said mixture and passing part of the residual sulfur dioxide to treat said one portion and passing another part to treat the pyrrhotite from second portion, uniting the magnetite thus produced and fluidizing it with an oxygen-containing gas to convert it to ferric oxide, returning a portion of said ferric oxide to the combined pyrrhotite, whereby the treatment of pyrrhotite is the sole source of sulfur dioxide in the system, and recovering ferric oxide.

3. That method of roasting pyrites to produce sulfur and ferric oxide comprising fluidizing one portion of pyrites with nitrogen-containing gas substantially free from oxygen at a temperature to drive off the labile sulfur atom and form pyrrhotite, separately fluidizing a

second portion of pyrites in the same manner, recovering the sulfur from said treatments, fluidizing the pyrrhotite from said one portion with an oxygen-containing gas at a temperature to convert it to magnetite and produce sulfur dioxide, treating the pyrrhotite from said second portion with sulfur dioxide, including that from said one portion, at a temperature and with fluidization to convert it to magnetite with production of a mixture of sulfur dioxide and sulfur vapor, condensing sulfur from said mixture and passing the residual sulfur dioxide to a heater, passing sulfur dioxide from the heater to treat said one portion and another part to treat the pyrrhotite from said second portion, uniting the magnetite thus produced and fluidizing it with an oxygen-containing gas to convert it to ferric oxide, and recovering the ferric oxide.

4. That method of roasting pyrites comprising the steps of fluidizing pyrites with non-oxidizing gas at a temperature to drive off the labile sulfur atom and form pyrrhotite, recovering the sulfur thus produced, dividing said pyrrhotite into two portions, fluidizing one of said portions with sulfur dioxide at a temperature to form magnetite and a mixture of sulfur dioxide and sulfur vapor, recovering sulfur from said mixture and passing part of the sulfur dioxide to treat said one portion and another part to fluidize the other of said portions at a temperature to produce magnetite and a mixture of sulfur dioxide and sulfur vapor, recovering sulfur from said last-named mixture, combining the magnetite thus produced and fluidizing it with an oxygen-containing gas at a temperature to convert it to ferric oxide, and recovering the ferric oxide.

5. That method of roasting pyrites comprising the steps of fluidizing pyrites with non-oxidizing gas at a temperature to drive off the labile sulfur atom and form pyrrhotite, recovering the sulfur thus produced, dividing said pyrrhotite into two portions, fluidizing one of said portions with sulfur dioxide at a temperature to form magnetite and a mixture of sulfur dioxide and sulfur vapor, recovering sulfur from said mixture and passing part of the sulfur dioxide to treat said one portion and another part to fluidize the other of said portions at a temperature to produce magnetite and a mixture of sulfur dioxide and sulfur vapor, recovering sulfur from said last-named mixture, combining the magnetite thus produced and fluidizing it with an oxygen-containing gas at a temperature to convert it to ferric oxide, and supplying said

5  
10  
15

sulfur dioxide solely by returning a portion of said ferric oxide to the combined magnetite to react with pyrrhotite with production of magnetite and sulfur dioxide, and recovering the ferric oxide.

6. That method of roasting pyrites comprising the steps of fluidizing pyrites with non-oxidizing gas at a temperature to drive off the labile sulfur atom and form pyrrhotite, recovering the sulfur thus produced, dividing said pyrrhotite into two portions, fluidizing one of said portions with sulfur dioxide at a temperature to form magnetite and a mixture of sulfur dioxide and sulfur vapor, recovering sulfur from said mixture and passing part of the sulfur dioxide to treat said one portion and another part to fluidize the other of said portions at a temperature to produce magnetite and a mixture of sulfur dioxide and sulfur vapor, recovering sulfur from said last-named mixture, combining the magnetite thus produced and fluidizing it with air at a temperature to convert it to ferric oxide and in an amount such that the off-gas is substantially oxygen free, passing said off-gas to fluidize said pyrites, and recovering the ferric oxide.

7. That method of roasting pyrites comprising the steps of fluidizing pyrites with non-oxidizing gas at a temperature to drive off the labile sulfur atom and form pyrrhotite, recovering the sulfur thus produced, dividing said pyrrhotite into two portions, fluidizing one of said portions with sulfur dioxide at a temperature to form magnetite and a mixture of sulfur dioxide and sulfur vapor, recovering sulfur from said mixture and passing part of the sulfur dioxide to treat said one portion and another part to fluidize the other of said portions at a temperature to produce magnetite and a mixture of sulfur dioxide and sulfur vapor, recovering sulfur from said last-named mixture, combining the magnetite thus produced and fluidizing it with air at a temperature to convert it to ferric oxide, said air being in an amount such that the off-gas is substantially oxygen free, passing said off-gas to fluidize said pyrites, supplying said sulfur dioxide solely by returning a portion of said ferric oxide to the combined magnetite to react with pyrrhotite to form magnetite and sulfur dioxide, and recovering ferric oxide.

45  
30  
35  
40  
45

References Cited in the file of this patent  
UNITED STATES PATENTS  
1,941,592 Bacon et al. ----- Jan. 2, 1934